

## 1

3,411,897

**METHOD FOR CONTINUOUS CASTING OF  
RIMMING STEEL**  
Paul E. Lindberg, Jr., Grosse Ile, Mich., assignor, by  
mesne assignments, to Concast Incorporated, New York,  
N.Y., a corporation of Delaware  
No Drawing. Filed Sept. 8, 1965, Ser. No. 485,915  
7 Claims. (Cl. 75—129)

### ABSTRACT OF THE DISCLOSURE

This is a method of partially deoxidizing molten steel to prepare rimming steel to be continuously cast. Vanadium is added to molten steel in an amount not more than about 82.50 pounds per 47 tons of molten steel. Thereafter not more than a total of about 50 pounds of aluminum are added per 47 tons of the molten steel, the aluminum being added a portion at a time to a point at which the customary agitation of the molten steel is without boiling and frothing when the steel is poured. The molten steel is then continuously cast by pouring it in one end of an open-ended mold and withdrawing a partially solidified casting from the other end.

This invention relates to the continuous casting of steel and, more particularly, to the continuous casting of rimming steel.

In the continuous casting of steel, molten steel is poured into the upper end of a mold open at its bottom. The mold is cooled by a liquid, such as water, circulated in the mold walls. When pouring is commenced, the bottom of the mold is closed with a metal plug. The plug cools the molten metal and the metal fuses to the plug. The cooled mold cools the metal in contact with the mold causing the molten metal to solidify and form a skin or sheath around the molten metal in the mold. The plug is withdrawn from the bottom of the mold and the steel, fused to the plug, follows. A continuous slab or casting of steel is thus formed. The plug is later removed from the end of the slab.

The skin or sheath formed around the molten metal in the mold is relatively thin at the time the cast slab emerges from the bottom of the mold. The metal, still molten in the center of the slab, is contained in the slab by this skin. The slab is supported by rollers which contact the slab below the mold. Some of the rollers are driven to regulate the speed at which the slab leaves the mold.

After leaving the mold, the cast slab is cooled. As the slab is cooled, the molten metal in the slab progressively solidifies from the outer wall of the slab inwardly. The skin or wall of solid metal thickens until, finally, all the metal in the slab is cooled and solidified. The point where the entire slab is solidified is below the mold and may be thirty-five feet, or more, from the point where the slab leaves the mold. Thus, as the slab leaves the mold, and for a considerable distance below the mold, the skin of solid metal around the slab supports the molten metal in the slab. Obviously, if this skin should be ruptured, the molten metal will escape and considerable damage to operating equipment can result, to say nothing of failure to form the required slab.

Unlike the casting of ingots where the metal is confined

5

10

15

20

25

30

35

40

45

50

55

60

65

## 2

in a mold until solidified and undesired oxides and impurities migrate to the top and bottom of the ingot and can be cut from the ingot during rolling, in continuous casting these impurities remain in the cast. Among these is uncombined oxygen which, as the molten metal cools, reacts and escapes as a gas from the molten metal. This escaping gas agitates the molten metal. Where the gas fails to escape before the metal solidifies, a bubble or void of substantial size may be formed in the cast.

A substantial portion of the molten metal in continuous casting is cooled and solidified after the slab leaves the mold. Where the collecting gas can escape upward through the molten metal, the gas vigorously agitates, boils and froths the molten metal. Such vigorous agitation and boiling interferes with the desired cooling of the molten metal by the cooled mold wall and hinders proper formation of the skin of solid metal around the slab, vital to continuous casting. Failure of the skin to properly form results in a weak wall which cannot support the molten metal.

The uncombined oxygen can be removed from the metal before the continuous cast is poured. This can be accomplished by the addition of materials to the molten metal which will react with, and absorb, all or substantially all of the uncombined oxygen.

Where rimming steel is to be formed, however, a controlled amount of uncombined oxygen is required. To obtain the necessary rimming action, through controlled agitation of the molten metal in the continuous cast, a certain amount of uncombined oxygen is desirable in the molten metal. This uncombined oxygen reacts to form a gas which moves through the molten metal and agitates the metal. By regulating the uncombined oxygen, the agitation or movement of the molten metal can be controlled so that the metal is agitated in a pattern in the mold. Thus, a cast of relatively dense, pure metal solidifies from the surface of the cast inwardly and impurities are moved away from the surface of the cast.

Attempts to adapt ingot casting deoxidation techniques for rimming steel to continuous casting have met with limited success and have resulted in the formation of relatively thin rimmed areas, high proportions of oxide impurities and casts which, when rolled, produced rolled sheets with streaks and flaws on, or close to, the surfaces of the sheets.

One of the objects of the instant invention is to provide an improved method for continuous casting of rimming steel.

A further object is to provide such a method that will form a relatively thick rimmed area.

A further object is to provide such a method wherein impurities in the cast are moved away from the surface of the cast.

Still a further object is to provide a continuous cast which can be rolled into relatively thin sheets without impurities or flaws on the surfaces of the sheets.

These and other objects will be more apparent from the following description:

In the instant method the metal for casting is prepared in the customary manner, is poured into a ladle and, from the ladle, is poured into the tundish of the continuous casting mold. At the time the metal is ready for pouring into the ladle, the iron oxide content of the slag is measured in accordance with customary practices.

The molten metal is poured into the ladle at a temperature of about 2950° to 3060° F. Difficulties in sampling, and the time available, do not allow precise measurement of the iron oxide content of the slag. However, and as will be more apparent from the following description, such measurement has been found sufficient for purposes of the instant invention. In addition to measuring the iron oxide content of the slag, the carbon, manganese, phosphorus and sulfur content of the metal are also measured. These later measurements are primarily for the purpose of determining the additions to the metal which may be required to produce the desired steel but may have an indirect relationship to the oxygen content.

The following description is based on an average charge of 47 tons of molten metal. Any substantial change in weight would, of course, lead to corresponding changes in the ladle additions to be described.

For rimming purposes, it is desirable to control the carbon content of the molten metal to be cast. The initial carbon content of the molten metal is regulated by the oxygen blowing of the metal. This blowing is adjusted so that the carbon content of the molten metal, when ready for pouring for low carbon rimming steel, does not substantially exceed 0.07%. Where higher carbon rimming steel is to be continuously cast, the blowing is adjusted for a higher carbon content. Where excess carbon is present, oxygen blowing is continued until the carbon content is reduced.

Where the carbon content of the metal is 0.07% or less, ten pounds of carbon, in the form of breeze, are added to the ladle as the metal is poured. If the metal has been over oxidized and the carbon content is substantially less than 0.05%, carbon addition may be increased to twenty pounds.

Carbon added to the molten metal, whether as breeze or in alloy additions, does, to a certain extent, react with and remove as a gas some of the uncombined oxygen in the molten metal. The amount of carbon that can be added, however, is limited. Thus, in the instant invention, the balance of the uncombined oxygen removed to attain a substantial uniform pattern of agitation in the molten metal during continuous casting and, at the same time, avoid excess agitation, boiling and froth in the mold and cast is removed by reaction with vanadium and aluminum additions to the molten metal.

Aluminum is well-known as a deoxidant in steelmaking. The aluminum combines with the uncombined oxygen forming aluminum oxide. In ingot casting of rimming steel, the aluminum oxide, which when formed is an impurity, migrates to the top of the ingot and is cut from the ingot during rolling. Attempts, heretofore, to utilize aluminum as a deoxidant in continuous casting of rimming steel have resulted in erratic rimming, relatively thin rims, and the formation of relatively large agglomerates of aluminum oxide at or near the surface of the cast slab which, when the slab is rolled, resulted in streaks and flaws on the surfaces of the rolled sheet.

In the instant invention, it has been discovered that the formation of these agglomerates of aluminum oxide at or near the surface of the continuously cast slab can be avoided by utilizing a combination of vanadium and aluminum as the deoxidant. It has been further discovered that, when so used for this purpose, the amount of each material employed is critical to the formation of a well rimmed cast free of oxide flaws at or near the surface.

The amount of deoxidant addition depends, of course, on the oxygen content of the metal for which the iron oxide content of the slag in the steelmaking furnace provides a satisfactory estimate for present purposes.

Vanadium, in the form of ferro vanadium, has been found to be acceptable. In the following description and examples ferro vanadium having an average analysis of 55.00% vanadium, 4.00% silicon, 2.50% carbon, and the balance iron is employed.

In carrying out the instant invention, it has been discovered that the amount of ferro vanadium and aluminum which can be added to the molten metal can be varied over a wide latitude. However, there is a limit on the maximum amount of each material that can be added and still obtain the desired results. For example, it has been found that the addition of more than 150 pounds of ferro vanadium (82.50 pounds vanadium) to a 47 ton melt does not produce the desired results. Likewise, it has been found that the addition of more than 50 pounds of aluminum does not produce the desired results. Within these maximum limits, however, the amounts added can be varied provided, of course, that a sufficient amount of the combined materials is added to attain the required deoxidation.

In the practice of the invention, the ferro vanadium is added to stabilize the melt and the aluminum to control the rimming action. The amount of ferro vanadium to be added to a particular melt is determined from the iron oxide content of the slag and the chemistry of the metal. It is preferred to add the ferro vanadium in a fixed amount and to vary the aluminum addition to suit the needs of the particular melt. For example, seventy-five pounds of ferro vanadium are added to the 47 ton melt and sufficient aluminum is added to reduce the uncombined oxygen content of the melt to the desired level. Where the measured iron oxide content of the slag is measured as 16% or less, seventy-five pounds of ferro vanadium is sufficient to maintain the required addition of aluminum well under the 50 pound limit. Where the iron oxide measurement exceeds 16% the ferro vanadium addition may be increased to one hundred pounds if it is desired to maintain the aluminum addition at a low level.

In the process of the instant invention, the vanadium apparently acts as a buffer and lowers the uncombined oxygen content of the molten metal to a point where it can be effectively controlled by the aluminum addition. Final control of the uncombined oxygen content is regulated by the aluminum addition. Because the measurement of the iron oxide content of the slag and the residual elements in the metal are not precise measurements, and the amount of uncombined oxygen in the metal may not have been precisely determined, the ferro vanadium is first added to the ladle. The aluminum is then added and the amount of aluminum is determined, to some extent, by the activity of the tapping stream and the metal in the ladle.

One method which has been found effective for regulating the aluminum addition and at the same time attaining the desired results of the instant invention, is to estimate the amount of aluminum required from the iron oxide measurement and the ferro vanadium addition and then add a portion of the estimated aluminum. If the metal in the ladle is relatively calm, is not excessively boiling and there is no frothing, the remaining portion is not added. If, on the other hand, the metal in the ladle remains wild, boils excessively and froths, the additional aluminum is then added. In some instances, even after the addition of the remaining portion further addition of aluminum may be required to reduce the activity of the metal in the ladle.

The melt for continuous casting is prepared at a temperature of about 2950° to 3060° F. The temperature of the melt in the ladle is about 2850° to 3000° F. and the temperature in the tundish, as the molten metal is being delivered to the continuous casting mold is about 2800° to 2875° F. As the temperature drops the molten metal may become more active and the activity may exceed that necessary for good and effective rimming. Where such activity occurs, additional aluminum may be added in the tundish. Usually, however, tundish addition is not necessary and it is preferred to add all of the required aluminum to the ladle.

The following are examples of casts, continuously cast following the method and process of the instant invention.

tion. In each example an average charge of 47 tons of molten metal was employed.

| Cast | Preliminary Analysis |      |      | Ladle Additions |     |     |    |
|------|----------------------|------|------|-----------------|-----|-----|----|
|      | C                    | Mn   | FeO  | FeMn            | FeV | C   | Al |
| 1    | .060                 | .200 | 12.5 | 300             | 50  | 50  | 15 |
| 2    | .045                 | .120 | 18.2 | 425             | 100 | 10  | 35 |
| 3    | .050                 | .200 | 14.5 | 175             | 75  | 10  | 15 |
| 4    | .050                 | .250 | 17.7 | 300             | 75  | 10  | 25 |
| 5    | .055                 | .180 | 22.3 | 350             | 100 | 10  | 25 |
| 6    | .040                 | .120 | 20.9 | 350             | 100 | 15  | 30 |
| 7    | .050                 | .300 | 16.0 | 150             | 100 | 10  | 15 |
| 8    | .045                 | .230 | 16.8 | 600             | 75  | 100 | 20 |
| 9    | .035                 | .170 | 21.0 | 450             | 100 | 10  | 40 |
| 10   | .060                 | .330 | 13.1 | 250             | 75  | 10  | 30 |
| 11   | .045                 | .210 | 13.3 | 300             | 75  | 10  | 20 |
| 12   | .045                 | .200 | 13.5 | 300             | 75  | 10  | 30 |
| 13   | .045                 | .210 | 17.2 | 300             | 75  | 10  | 25 |
| 14   | .055                 | .280 | 12.5 | 200             | 75  | 10  | 25 |
| 15   | .045                 | .120 | 18.7 | 450             | 75  | 10  | 35 |
| 16   | .045                 | .240 | 16.5 | 250             | 75  | 10  | 15 |
| 17   | .050                 | .320 | 13.3 | 200             | 75  | 10  | 10 |
| 18   | .050                 | .180 | 13.2 | 250             | 75  | 10  | 20 |
| 19   | .055                 | .320 | 16.2 | 150             | 75  | 10  | 20 |
| 20   | .060                 | .220 | 19.4 | 400             | 75  | 10  | 25 |
| 21   | .070                 | .200 | 22.7 | 200             | 75  | -0  | 30 |
| 22   | .065                 | .260 | 19.2 | 250             | 75  | 10  | 20 |
| 23   | .070                 | .400 | 14.0 | 150             | 75  | -0  | 25 |
| 24   | .070                 | .390 | 14.0 | 150             | 75  | -0  | 20 |
| 25   | .045                 | .140 | 15.5 | 400             | 75  | 10  | 20 |
| 26   | .050                 | .240 | 20.9 | 250             | 75  | 10  | 25 |
| 27   | .050                 | .160 | 22.5 | 400             | 75  | 10  | 25 |
| 28   | .045                 | .310 | 16.5 | 200             | 75  | 10  | 15 |
| 29   | .060                 | .210 | 15.7 | 200             | 75  | -0  | 15 |
| 30   | .050                 | .270 | 17.3 | 150             | 75  | 10  | 20 |

NOTE.—C=carbon; Mn=manganese; FeO=ferrous oxide (calculated from total iron); FeMn=ferro manganese; FeV=ferro vanadium; Al=aluminum.

The terms and expressions which have been employed are used as terms of description and not of limitation, and there is no intention, in the use of such terms and expressions, of excluding any equivalents of the features shown and described or portions thereof, but it is recognized that various modifications are possible within the scope of the invention claimed.

What is claimed is:

1. A method of partially deoxidizing and continuously casting rimming steel comprising adding to molten steel not more than about 82.50 pounds of vanadium per 47 tons of molten steel, then adding not more than about 50 pounds of aluminum per 47 tons of molten steel, said aluminum being added a portion at a time to a point at which agitation of the molten steel is without vigorous

35

40

30

10

15

20

25

30

boiling and frothing when poured, thereafter continuously casting the steel by pouring it in one end of an open-ended mold wherein the periphery of the steel is solidified to form a casting having a molten core, withdrawing the casting from the mold as a continuous strand, and subsequently cooling the casting to solidify it completely with a rimmed structure.

2. The method of claim 1 in which the vanadium is ferro vanadium containing the specified amount of vanadium.

3. The method of claim 1 in which, when the slag on the molten steel, immediately before tapping, contains less than about 16% iron oxide, the amount of vanadium added is from about 27.50 pounds to about 41.25 pounds.

4. The method of claim 1 in which, when the slag on the molten steel, immediately before tapping, contains more than about 16% iron oxide, the amount of vanadium added is from about 41.25 pounds to about 82.50 pounds.

5. The method of claim 1 in which the amount of aluminum added is from about 10 pounds to about 50 pounds.

6. The method of claim 1 in which the amount of vanadium added is from about 27.50 pounds to about 82.50 pounds.

7. The method of claim 1 in which the amount of vanadium added is from about 27.50 pounds to about 55 pounds, and the amount of aluminum added is from about 10 pounds to about 40 pounds.

#### References Cited

##### UNITED STATES PATENTS

|           |         |                  |          |
|-----------|---------|------------------|----------|
| 1,420,328 | 6/1922  | McConnell        | 75—129   |
| 1,727,180 | 9/1929  | Saklatwalla      | 75—129 X |
| 2,221,781 | 11/1940 | Critchett et al. | 75—58    |
| 2,253,574 | 8/1941  | Norbeck          | 75—58    |
| 2,291,842 | 8/1942  | Strauss          | 75—58    |
| 2,360,271 | 10/1944 | Peterson         | 75—58 X  |
| 2,999,749 | 9/1961  | Saunders et al.  | 75—58    |
| 3,030,204 | 4/1962  | Staggers et al.  | 75—129   |

L. DEWAYNE RUTLEDGE, Primary Examiner.

H. W. TARRING, Assistant Examiner.